

E. SOKOLOWSKI.  
CAST EXPLOSIVE CHARGE;  
APPLICATION FILED MAY 15, 1912.

1,054,147.

Patented Feb. 25, 1913.



FIG. 1.

FIG. 2.

WITNESSES:

R. F. Litchel  
E. E. Hall

INVENTOR

Ernest Sokolowski  
BY Frank L. Buser  
ATTORNEY.

# UNITED STATES PATENT OFFICE.

ERNST SOKOLOWSKI, OF HAMBURG, GERMANY, ASSIGNOR TO E. I. DU PONT DE NEMOURS  
POWDER COMPANY, OF WILMINGTON, DELAWARE, A CORPORATION OF NEW  
JERSEY.

## CAST EXPLOSIVE CHARGE.

1,054,147.

Specification of Letters Patent. Patented Feb. 25, 1913.

Original application filed October 3, 1911, Serial No. 652,480. Divided and this application filed May 15, 1912. Serial No. 697,588.

To all whom it may concern:

Be it known that I, ERNST SOKOLOWSKI, a subject of the Emperor of Germany, residing at Hamburg, Germany, have invented a new and useful Improvement in Cast Explosive Charges, of which the following is a full, clear, and exact description, reference being had to the accompanying drawings, which form a part of this specification.

The ordinary cast fusible explosive exhibits certain characteristics which give rise to certain disadvantages which it is the object of my invention to eliminate. One of the most pronounced of these objectionable characteristics is the lack of a homogeneous loading. It has been observed, on cross-section of cast explosive charges, that during the act of solidification small cavities or hollow spaces are formed, especially along the longitudinal central portion of the explosive charge, said hollow spaces arising from the shrinkage of the fused mass in the process of chilling, which heretofore has been from the outer surface concentrically to the inside. It is clear that in the moment of the firing, when the gases of the smokeless powder impart the first impact to the projectile, the charge contained in the latter must undergo a kind of crushing, which will lead to compression and consequent friction in the case of the charge being compressible, *i. e.* not having its highest attainable density before the shot is fired. Moreover the hitherto used explosive charges show very often a relatively coarse crystalline structure, owing to the low cooling of the fused mass, even if placed during solidification in cold water. The long crystals thus formed are liable to break in the moment of the violent impact of the shot. Hence premature detonations of the projectiles may and do occur, which destroy both cannon and crew, and can only be avoided by eliminating friction within the shells. Furthermore, modern explosives are sometimes somewhat insensitive, and the detonation of the primer is then not easily propagated to the whole main charge, whereby the latter will often explode only partly. In order to offset this drawback, intermediate charges have been adopted, which act as propagators between the primer and the main cast explosive charge, but owing to the

length of modern projectiles these intermediate priming charges do not always perform their purpose, because they commonly surround the primer, thus being embedded in one end and too distant from the opposite end of the long cylindrical main charge which will often remain partly unexploded, notwithstanding the use of the intermediate priming charge.

The object of the present invention is to produce a cast fusible explosive charge in which the coarse crystalline structure above mentioned is absent and which instead exhibits an absolutely homogeneous fine crystalline structure of high density and devoid of hollow spaces and which cannot be further compressed by the impact of the shot, thereby avoiding both premature detonation and only partial explosion of the charge.

The invention consists of an explosive charge comprising a main body of explosive and an internal longitudinally extending explosive core tightly and permanently surrounded by the main body of the explosive.

In order that the invention may be fully understood, I will first describe the method which I have adopted for the manufacture of the charge.

Into the center line of the mold a cold substance made of an explosive in the shape of a rod is introduced and maintained in position by means of a suitable appliance from its upper end. The introduction of the cold rod made of an explosive substance can be effected in such manner that this rod is introduced into the empty mold before the fused material is poured into same, or the rod can be inserted after the cast has been made by pressing same into the latter. The filling of the mold may be carried out in accordance with any desired pouring process, for instance, by means of an ordinary casting, by means of casting under pressure, or by means of a heatable pouring funnel. In the latter case the neck of the funnel can be used for the guiding of the cold rod-shaped substance. The latter consists, for instance, of an explosive which is not covered and which has been fused and chilled, or of an explosive pressed in a tube-shaped closed shell, the latter, for instance, consisting of celluloid, pasteboard or sheet metal. The diameter of this cold, rod-shaped explo-

sive material is to be adapted to the diameter of the explosive charge. By means of providing this cold rod made of an explosive substance in the center of the cast, or 5 by sinking this rod into the fused explosive mass, a quick chilling of the liquid portion of the charge is effected. The rod-shaped cold explosive body is thus tightly surrounded by the chilling explosive charge. Experience shows that fusing of the rod substance does not take place, or takes place to 10 but a slight extent, whenever the casting operation is carried out at as low a casting temperature as possible and with indications 15 of the commencement of the formation of crystals. This condition is of great importance in this method of casting and for the purpose of producing the high density of the cast obtained thereby.

20 When using a rod made of a pressed explosive in a pasteboard or other cover, this pressed explosive serves directly as a priming charge, which tightly bears against the bottom of the explosive charge container 25 surrounding the igniting charge of the fuse. Owing to the long shape of this priming charge passing almost throughout the entire 30 length of the charge, the detonation becomes very satisfactory, and a very strong propagation 35 of the detonation upon the fused main charge is more fully insured than in the case of the usual priming charges placed with one side only near the fuse and surrounding the same. Of special importance is the advantage that, as a consequence of 40 the quick cooling of the cast simultaneously from the outside and from the inside, a very fine crystalline structure of the cast, and as high a density as possible, are obtained.

45 For this reason large crystals will not break, even though the impact of the shot should be especially violent, and the charge will not contract, since the highest possible density has been imparted to the same during the casting, and since a densifying beyond 50 this point is not possible. These two points render impossible movements within the explosive charge with a violent impact of the shot, thus directly insuring against premature detonations to an extent which is not obtained when using other pouring methods.

55 Of special importance is the fact that the explosive used for the cold rod-shaped body can possess chemical properties entirely different from those of the main charge. It is therefore possible to use, for the rod charge, for instance a brisant explosive which detonates with violence; while for the main charge a more inert fused explosive which 60 is very safe against shock, for instance trinitrotoluol, can be used.

65 Explosive charges embodying my invention, prepared in accordance with the above described method, when cut open, clearly show that they have been actually so pre-

pared, which guarantees to a high degree the good quality of the charge. When using, for instance, the rod-shaped body without a cover and made of a fused explosive, the structure of the same can be clearly distinguished from that of the main charge, since its appearance is different, notwithstanding the fact that an exceedingly intimate fusion of the two charges has been effected. This is, of course, still more apparent when the rod body is used in a pressed state and with a special cover.

70 In the drawings, Figures 1 and 2 are longitudinal sectional views of molds containing alternate forms of explosive charges 80 embodying my invention, Fig. 1 showing an uncovered explosive core and Fig. 2 an explosive core in a shell.

*a* represents an iron casting mold, *b* a paste-board container placed in the same, 85 and *c* (Fig. 1) a rod-shaped body of fused explosive extending throughout the axial length of the mold.

*c* (Fig. 2) represents a rod-shaped body 90 consisting of a paste board shell *d* with several pressed bodies of explosives, *c'*, placed therein.

*e* represents the main explosive body.

I do not herein claim the process by which the explosive charge forming the subject 95 matter of this application is manufactured, as the same forms the subject matter of an application heretofore filed by me, Serial No. 652,480, filed October 3, 1911, of which this application is a division.

100 I am aware that it has been proposed to make the explosive charges of projectiles less liable to premature detonation following internal friction by surrounding a central core of dynamite or other more sensitive explosive covered by absorbent material with a body of nitro-gelatin or other less sensitive explosive similarly covered; also to divide the loose main explosive charge into a number of sections supported 105 by shells, disks, webs, etc.; also to make the bursting charge of layers of dynamite cloth. But these charges are more or less compressible so that the danger of internal friction in the movement of the shot is not 110 altogether removed. In my invention, however, all danger of internal friction is removed by imparting to the explosive charge the highest attainable density so that it cannot be further compressed by the shock of 115 the projectile when the shot is fired or the target hit. Another important factor is the fine crystalline structure of the charge, which can be produced only by the process described in the application of which this 120 is a division.

125 Having now fully described my invention, what I claim and desire to protect by Letters Patent is:

1. A cast explosive comprising a main 130

body of a relatively dense and fine crystalline explosive in the form of a solid block surrounding a longitudinally extending central core of a less dense and previously chilled explosive and therefore adapted during the casting to help control the crystalline structure and density of the main body.

2. A cast explosive comprising a main explosive body consisting of a solid block and to an internal uncovered explosive core di-

rectly and integrally united with the main body.

In testimony of which invention, I have hereunto set my hand at Hamburg, on this 26th day of April, 1912.

ERNST SOKOLOWSKI.

Witnesses:

ERNEST H. L. MUMMENHOFF,  
IDA CHRIST HAERMAN.